

## UNITED STATES PATENT OFFICE

2,213,343

## ELECTRIC CONTACT COMBINATION

Franz R. Hensel and Kenneth L. Emmert, Indianapolis, Ind., assignors to P. R. Mallory & Co., Inc., Indianapolis, Ind., a corporation of Delaware

No Drawing. Application February 20, 1940,  
Serial No. 319,888

4 Claims. (Cl. 200—166)

This invention relates to electrical contacts.

An object of the invention is to improve the combinations of compositions for electrical make and break contacts.

Another object of the invention is to provide a contact combination which can be operated without objectionable contact metal transfer in automobile electrical systems.

A still further object is to provide a contact metal combination which will retain a low contact resistance.

Other objects of the invention will be apparent from the following description, taken in connection with the appended claims.

The present invention comprises a combination of elements, methods of manufacture and products thereof, brought out and exemplified in the disclosure hereinafter set forth, the scope of the invention being indicated in the appended claims.

While a preferred embodiment of the invention is described herein, it is contemplated that considerable variation may be made in the method of procedure and combination of elements, without departing from the spirit of the invention.

Up to the present time, electrical contacts which are used, particularly for such applications as ignition systems, are made from pure tungsten and it is generally understood that the highest purity tungsten will give the best contact performance, particularly as far as metal transfer is concerned.

We have found that we can improve upon the contact performance of pure tungsten in D. C. circuits, particularly automotive ignition circuits, by providing a differential contact combination, wherein the positive contact consists of pure tungsten (at least 99.9% tungsten) and the negative contact consists of an alloy of tungsten and molybdenum.

We have found that binary alloys of tungsten and molybdenum show an increased hardness and therewith resistant to mechanical abrasion. At the same time they have shown considerable resistance to material transfer or build-up. We are aware of the fact that tungsten-molybdenum alloys, however, have been previously made for a number of purposes. The alloys, have, however, never obtained any commercial importance in the field of electrical contacts, due to the fact that higher molybdenum contents have a tendency to produce excessive contact resistance values. This was particularly noticeable if the molybdenum content exceeded 10%.

Tests have been run on tungsten contact combinations, where the positive contact consisted of

pure tungsten, having a grain count of approximately 40,000 to 50,000 grains per square millimeter, and the negative contact consisted of a tungsten-molybdenum alloy which in the preferred case had a composition of 99.75% tungsten and .25% molybdenum. The grain size of the alloy varied from approximately 10,000 to 30,000 grains per square millimeter.

Standard comparison tests on several automotive ignition systems were conducted, wherein the distributor was operated at cam speeds of from 550 to 750 R. P. M., with a primary applied voltage of 8.5 volts at a primary peak current of 5.4 to 5.7 amperes, the contact or primary gap spacing being .020, with secondary gap spacing of .375", which secondary gap discharged in air, the duration of these tests being in the order of 650 to 1000 continuous operating hours.

Based on the above testing procedure, a standard tungsten versus tungsten combination of the prior art gave an operating efficiency of from 70 to 75% determined by measuring the area under the curve produced by plotting the number of satisfactory units in operation versus time, while the combination of the present invention, based on the same method of comparison, gave efficiency values of from 90 to 96%. (Note: A rating of 100% on the above test would be produced by all units starting a test and operating satisfactorily, both from the standpoint of metal transfer and contact resistance for the total duration of the test.)

It has also been found that the combination of the present invention is much superior to a contact combination of tungsten-molybdenum alloy versus tungsten-molybdenum alloy. The operating efficiency, with the alloy used for both contacts was found to be 25 to 30% lower than the combination of the tungsten-molybdenum alloy versus pure tungsten. Moreover, if the polarity is reversed so that pure tungsten is used for the negative contact and tungsten-molybdenum alloy for the positive contact the efficiency obtained is 20 to 40% below that of the combination contemplated by the invention.

Tests of the type described were carried out regularly over the period of nearly a year and have confirmed that, on electric systems wherein material transfer or build up is the main factor to be considered, the application of the combinations contemplated by the present invention will produce operating characteristics far more satisfactory than was possible with prior art conditions.

In D. C. circuits, the positive contact or the

anode generally tends to oxidize more quickly and more severely than the cathode. This condition of over-oxidization is experienced in ignition systems when operated at low temperatures. The 5 oxidation under these conditions is primarily due to increased burdens across the contact points, caused by radical reduction in coil resistance values. Furthermore, there seems to exist certain electrochemical reactions, causing a certain 10 type of anodic oxidization. The contact combinations of the present invention were tested in systems operating in cold boxes at  $-10^{\circ}$  F. and were found 100% satisfactory for periods in excess of 500 continuous hours of operation, whereas 15 contacts of the prior art such as tungsten versus tungsten had numerous failures under the same conditions.

The tests were extended to materials having considerably higher molybdenum contents and in 20 some cases, the molybdenum was raised up to 10%. By adjusting to electrical circuit conditions, it was possible to obtain the improved contact performance with a combination having as one contact a tungsten-molybdenum alloy containing up to 10% molybdenum.

The contact combinations containing molybdenum in percentages up to 10% were found very satisfactory for direct current applications, where the potential was in the order of 24 to 110 volts. 30 In arriving at the best possible combinations, also the quality of the pure tungsten was varied and materials were used of different grain counts, varying from a grain count of 10 grains per square millimeter up to 100,000 grains per square 35 millimeter. Also materials were tried on the pure tungsten side which had received special heat treatments, such as low temperature anneals in a hydrogen atmosphere. It was found that the various pure tungsten materials could be satisfactorily applied, providing that the purity of the tungsten was high enough. The tests indicated, however, that the most satisfactory performance 40 of this new combination was obtained with a pure tungsten of a comparatively small grain size.

45 The tungsten-molybdenum alloy according to the invention may have a permissible range of composition of

Molybdenum ..... per cent .05 to 10  
Tungsten ..... balance

Most of the preferred compositions will have a molybdenum content of .05 to 2.5% and more preferably from .1 to .5%.

The tungsten-molybdenum alloys may be produced by well known and standard methods such as by sintering the metal powders together, and alternately swaging and heat treating. 5

While the present invention as to its objects and advantages has been described herein as carried out in specific embodiments thereof, it is 10 not desired to be limited thereby, but it is intended to cover the invention broadly, within the spirit and scope of the appended claims.

What is claimed is:

1. An electric contact combination for D. C. 15 operation in automotive ignition circuits, the contact on the positive side of said combination being pure tungsten and the contact for the negative side being formed from an alloy of tungsten and molybdenum containing .05 to 10% of molybdenum. 20

2. An electric contact combination for D. C. 25 operation in automotive ignition systems, the contact on the positive side of said combination being pure tungsten and the contact for the negative side being formed from an alloy of tungsten and molybdenum, containing .1 to .5% molybdenum.

3. An electric contact combination for D. C. 30 operation in automotive ignition systems, the contact on the positive side of said combination being pure tungsten and the contact for the negative side being formed from an alloy of tungsten and molybdenum, containing .25% molybdenum.

4. In an automobile electrical system, a direct 35 current make and break contact combination comprising a contact of tungsten on the positive side and a cooperating contact of tungsten containing from approximately .05 to 2.5% molybdenum on the negative side, said contact combination being capable of operation in low temperatures without excessive oxidation and metal transfer. 40

FRANZ R. HENSEL.  
KENNETH L. EMMERT.

45